

Jan. 6, 1959

W. H. BRAUN, JR.

2,867,543

WOOD IMPREGNATING AND COLORING PROCESS

Filed Oct. 22, 1956

FIG. 1.



FIG. 2.



WILLIAM H. BRAUN, JR.,  
INVENTOR.

BY  
William P. Green  
ATTORNEY.

1

2,867,543

## WOOD IMPREGNATING AND COLORING PROCESS

William H. Braun, Jr., North Hollywood, Calif., assignor to Western Sealant Development Corporation, Culver City, Calif., a corporation of California

Application October 22, 1956, Serial No. 617,224

14 Claims. (Cl. 117—46)

This invention relates to improved processes for treating wood in a manner to vastly improve its physical characteristics, and also at the same time, to improve and control its general appearance. As will appear, these results are attained by a unique process in which the wood is impregnated with a resinous plastic material, which resin is cured after impregnation into the wood, and with the overall process being controlled to produce the desired change in the appearance of the wood.

When cured, the resin forms a strong and hard lattice-like structure extending into the pores of the wood and coating its surfaces, and giving the wood greatly increased strength and hardness. This increased strength and hardness, together with the above discussed controlled change in appearance, render it possible to utilize soft woods, such as pine, fir, spruce and redwood, etc., for purposes ordinarily requiring expensive hard woods. The use of such soft woods in the place of hard woods has the obvious advantage of reducing costs, and also greatly simplifies the process of machining or shaping the wood, for example in making furniture, since the soft woods can be shaped very easily prior to impregnation, and can then be readily converted to an altered very hard and strong state by the impregnation process. After the impregnation, the surface of the wood may be sanded or otherwise worked, and requires no varnishing or other surface coating by reason of the presence of the plastic in the wood.

In addition to increasing the strength and hardness of the wood, the present process also renders the composite wood and plastic structure much more uniform throughout, since the plastic very effectively fills in all cracks, crevices, and other voids in the wood. Further, the treatment increases, by approximately ten times, the resistance of the wood to water absorption, and also considerably increases the resistance to fire, chemical attack, and other types of damage or deterioration.

The present invention is in certain respects particularly concerned with the control of the process in a manner to darken the color of the wood during the process, so that an initially light-colored and inexpensive wood may have the appearance of a dark and normally very rare, expensive wood. For instance, a low-cost, light-colored wood may be given the appearance, as well as the physical characteristics, of such woods as ebony, teakwood, ironwood, and the like. In addition, the process may be very easily regulated to produce any intermediate shade of wood between the very lightest and the very darkest to thereby produce various attractive appearances not hitherto known, and to accomplish all of these different appearances without changes in the resinous material being used as an impregnant. Thus, a single batch of resin may be employed for forming impregnated woods of various different colors at will, with the result that a commercial application of the invention can, without un-

2

due expense, be extremely flexible as to the type and color of product being produced from a single impregnating unit.

To attain such color control, the process is designed 5 to actually change the color of the wood itself, as distinguished from the resin which impregnates the wood. The resin is then so chosen as to be light-passing in character, so that the changed color or shade of the wood is visible through the resin. Preferably, the cured resin 10 is transparent or clear, and desirably substantially colorless, to allow viewing through the resin of the darkened grain structure and highlights of the wood, with the result that the overall appearance of the wood may be extremely attractive. If desired, in order to achieve a 15 particular effect, the cured resin may, in some cases, be translucent rather than transparent.

In accordance with the invention, the change in color of the wood is effected by heating the wood to an extent (at a temperature and for a time) sufficient to visibly 20 and considerably darken the color of the wood, by virtue of the internal reactions which occur in the wood as a result of the heating. It is, of course, virtually impossible to define exactly what types of reactions produce this 25 darkening action, but for present purposes, it will suffice to say, merely that the heat appears to cause changes in the organic materials in the wood which visibly change the color of the wood. To produce a visible change in the wood color, the heat must be considerably greater than that normally utilized and required for curing of the 30 resin. The extent to which the wood is darkened may be controlled by regulating the amount of heat to which the wood is subjected, so that the wood may be given either a light brown or tan appearance, or a dark, almost black, appearance, or any intermediate appearance or shade.

The heat and the temperature to which the wood is subjected should, at a minimum, be at least enough to visibly darken the wood, and should, at a maximum be less than the temperature and heat which would break down or 40 damage the resin being used, and less than the char point of the resulting composite wood and resin product. To make a commercially practical operation, the temperature for darkening the wood is preferably at least about 350° F., and preferably not greater than about 475° F. The optimum temperatures for certain specific woods are as follows:

Pine, between about 350° F. and 400° F.;  
Fir, between about 375° F. and 425° F.; and  
Birch, between about 380° F. and 430° F.

When the temperatures are within the range of 350° F. to 475° F., the darkening of the wood may be produced within commercially practicable time periods, usually between about ½ hour and 2 hours.

For best results, I find it most desirable, in performing the process, to first evacuate all air and volatile materials from the pores of the wood, then to impregnate the uncured resin into the pores of the wood, then to cure the resin (usually by heat), and then to further heat the wood and resin to an extent visibly darkening the color of the former but not damaging the resin (preferably at a temperature between 350° F. and 475° F. as discussed).

As mentioned above, the wood is preferably so treated, prior to its actual impregnation, as to evacuate as much as possible of the air and volatile constituents from the pores of the wood, so that a maximum amount of resin may be forced into those pores. Such evacuation is effected by subjecting the wood to a relatively high vacu-

um, usually amounting to an absolute pressure of less than 30 mm. Hg, (preferably under 5 mm. Hg). The evacuation may be further enhanced by maintaining the wood at an elevated temperature during its subjection to the vacuum, the temperature typically being at least about 120° F. but under the kindling temperature of the wood, and preferably being between about 200° F. and 350° F. (optimum about 250° F.).

After the air and volatile constituents have thus been driven out of the pores in the wood, the uncured resin in liquid form may then be forced by pressure into those pores to deeply impregnate the wood. Such impregnation may be effected by completely immersing the wood in a body of the liquid resin, and then subjecting the resin to superatmospheric pressure to force it into the wood. The pressure may be about 100 p. s. i., and may be alternately applied and relieved through one or more cycles (normally 2 to 5 cycles), to effect a more thorough impregnation than can be attained by a single application of pressure. Between the pressure periods, the pressure of the resin and therefore of the wood may be reduced only to atmospheric pressure, or may actually be reduced to a vacuum, say as low as  $\frac{1}{2}$  p. s. i. absolute, and preferably less than 5 mm. Hg. Apparently, this alternate application of superatmospheric and then subatmospheric pressure acts to first force the resin partially into the wood, and then to allow small amounts of retained air and gases to bubble out through the resin (while under vacuum), following which another pressure surge forces the resin more deeply into the pores, etc. It has been found that in this way the resin can be forced into the pores of the wood through its entire thickness, so that the resulting product may be of substantially uniform composition throughout.

The resin employed is preferably a thermosetting resin, as for instance, a polyester resin, an epoxy resin, a phenol formaldehyde resin, or a urea formaldehyde resin. Typical examples of particular commercial resins which may be employed are the following:

(1) The polyester resin sold under the trade name P. E. 1 by Western Sealant Development Corp., 9999 West Jefferson Boulevard, Culver City, California.

(2) The epoxy resin sold as Epon #828 by Shell Development Corp., 1008 W. 6th St., Los Angeles, California.

(3) The phenol formaldehyde resin sold as BLL-3085 by Union Carbide & Carbon Corp., 2770 Leonis Street, Vernon, California.

(4) The urea formaldehyde resin sold as Uformite #700 by Rohm & Haas, 5657 Wilshire Boulevard, Los Angeles, California.

The resin is, in some cases, mixed with a suitable diluent, such as styrene monomer or phenylglycidal ether, and may contain an additive or additives to increase its speed of curing, or to give other desired characteristics, certain typical additives being benzoyl peroxide, diethylene triamine or dodecylsuccinic acid anhydride.

Following the impregnation of the resin into the wood, the wood may be removed from the body of liquid resin within which it is immersed, and excess resin may be cleaned from its outer surface by a brush, squeegee, the application of solvent, or any other suitable method. However, sufficient resin is left on the outer surfaces of the wood to form a thin coating of resin on those surfaces as well as in the pores.

The next step is to cure the thermosetting resin, usually by baking in a suitable oven. The curing temperature and time may be as prescribed by the manufacturer of the particular resin employed, but for most resins (including those specifically enumerated above) a curing temperature of 250° F. for one hour will be satisfactory.

The wood-darkening operation may be performed as a final step in the process, which, in some cases, may occur in its entirety after the curing of the resin has been completed. In other cases, however, the darkening of

the wood may be commenced during the actual curing step itself, if the curing temperature is purposely made considerably higher than that normally prescribed for curing, and is sufficiently high to actually commence the darkening of the wood; that is, the temperature in the curing oven may, from the outset, be within the range previously prescribed for most effective darkening of the wood (350° F. to 475° F.), in which case the resin will very rapidly cure (say in about 30 minutes), with little or no darkening of the wood in that short period. After such curing, the continued heating of the wood and resin at this high temperature will produce a very readily visible and progressive darkening of the wood until a desired shade has been attained. If the initial curing is at a conventional relatively low curing temperature, such as 250° F., the temperature must be raised after completion of the curing to a value such as that previously discussed which will produce the desired visible color change.

The apparatus for performing the present process may be completely conventional, and therefore will not be described in detail in this application. The initial evacuation and impregnation may be performed in a conventional autoclave, within which the wood may be placed, and which can first be subjected to an internal vacuum, then be filled with resin through suitable piping, then be subjected to pressure and vacuum alternately to force the resin into the wood, and finally be drained to allow removal of the wood. The baking and heat treating can of course be performed in any furnace capable of raising the wood and resin to the specified temperatures.

To assure the adequacy of the present disclosure, the following typical examples are given of specific processes embodying the invention:

#### Example 1

A piece of white pine measuring 4" x 6" x 1" was placed in an autoclave, and the autoclave was then closed and sealed. A connected vacuum pump was then placed in operation to reduce the pressure in the autoclave and about the wood to 3 mm. Hg, and the autoclave and wood were simultaneously heated to 120° F. After this pressure and temperature had been maintained for 1 hour, a liquid resin solution was admitted into the autoclave to a level completely immersing the wood, the solution consisting of:

128 parts polyester resin as sold by Western Sealant Development Corporation under the trade designation P. E. 1.

55 parts styrene monomer

1 part benzoyl peroxide

The vacuum was then relieved and the resin solution was subjected to a pressure of 100 p. s. i. for 60 minutes, following which the pressure was reduced to a vacuum of 3 mm. Hg for 15 minutes and this cycle was then repeated 3 times to force the liquid resin into the pores of the wood throughout its thickness. Next the resin was drained from the autoclave, and the wood was removed. The excess resin was cleaned from the outer surfaces of the wood by brushing, but leaving a thin layer over the entire surface of the wood.

After cleaning, the impregnated wood was placed in an oven and heated for one hour at 250° F. and at atmospheric pressure to thoroughly cure the thermosetting resin. Following the curing period, the temperature was raised to 350° F. for a period of 1 hour, to darken the color of the wood to a golden brown color, without substantially affecting the transparent appearance of the resin. The product made in this way was hard, strong, fire-resistant, chemical-resistant, water-resistant, and of a uniform darkened color throughout its thickness. It did not require varnishing or other protection, and could be sanded or cut to any shape without affecting its surface color or finished appearance.

*Example 2*

Same process as that of Example 1, except for the following variations:

- (1) Fir wood instead of pine
- (2) Composition of resin solution

704 parts epoxy resin as sold by Shell Development Corporation under the trade designation Epon 828

32 parts phenyl glycidal ether

1 part diethylene triamine

192 parts dodecylsuccinic acid anhydride

(3) Curing temperature 300° F. for 45 minutes.

(4) Temperature raised to 400° F. for 1/2 hour after curing period to darken wood.

*Example 3*

Same process as Example 1, except for following variations:

(1) Birch instead of pine

(2) Resin composition: 100% phenol formaldehyde resin, sold as BLL-3085 by Union Carbide and Carbon Corporation.

(3) Curing temperature 300° F. for 45 minutes.

(4) Elevation of temperature to 400° F. for 1/2 hour after curing, to darken wood.

*Example 4*

Same as Example 1, except temperature raised to 400° F. at commencement of curing and for 1 hour to first cure the resin at that temperature in about 30 minutes and then continue the heating after curing to darken the wood.

To facilitate an understanding of the present invention, there is submitted herewith a drawing, in which:

Fig. 1 is a fragmentary cross-sectional view taken through a piece of impregnated wood 10 which has been formed in accordance with the invention; and

Fig. 2 is a flow-sheet representation of a preferred process embodying the invention.

In Fig. 1, the final product 10 includes a piece of wood represented at 11, and which is continuously coated along all of its outer surfaces by a layer of cured thermosetting resinous plastic material 12. This cured resin also extends deeply into the pores of the wood, preferably throughout its entire thickness. The wood has been darkened in color by heating, and the resin is of a light passing-character allowing viewing of the darkened color of the wood through outer resinous layer 12.

As represented in the flow sheet of Fig. 2, the first step in the preferred process may be to evacuate the pores of the wood, preferably by a combination of heat and subjection to vacuum. The next step is then to impregnate the wood with uncured thermosetting resin, following which the resin is cured as step three. Finally, the wood is darkened, as discussed in great detail above, by heating the wood after the curing step.

I claim:

1. The method of producing an impregnated darkened wooden member that comprises evacuating air and volatile constituents from the pores of a piece of wood by heating the wood and subjecting it to a vacuum, then immersing said wood in a body of uncured thermosetting resin in liquid form, applying pressure to said resin and thereby forcing the resin into the pores of the wood, removing said wood from the body of resin with some of the resin retained in the pores of the wood and coating the surface of the wood, heating said wood and carried resin and thereby curing the latter to a hardened polymerized form, and then continuing the heating of said wood and carried resin after the latter has been cured to said hardened form and for a time and at a temperature sufficient to visibly darken the color of the wood by heat after said curing but not sufficient to break down the cured resin,

said cured resin being transparent to allow the darkened grain of the wood to be visible therethrough.

2. The method of producing an impregnated darkened wooden member as recited in claim 1, including alternately applying pressure and vacuum to said body of resin while the wood is immersed therein to thereby cause deep penetration of the resin into the wood.

3. The method of producing an impregnated darkened wooden member as recited in claim 2, in which said darkening of the wood is effected at a temperature between about 350° F. and 475° F.

4. The method of producing an impregnated darkened wooden member that comprises impregnating a piece of wood with a thermosetting resin by forcing said thermosetting resin under superatmospheric pressure into the pores of the wood, curing said thermosetting resin to a hardened polymerized state after its impregnation into the wood, and heating said wood and resin after the resin has been hardened and for a time and at a temperature sufficient to visibly darken the color of the wood by heat after curing but not sufficient to break down the hardened cured resin, said resin being of a light-passing character allowing the darkened color of the wood to be visible therethrough.

5. The method of producing an impregnated darkened wooden member as recited in claim 4, in which said darkening of the wood by heat is effected at a temperature at least as high as high as about 350° F.

6. The method of producing an impregnated darkened wooden member as recited in claim 4, in which said darkening of the wood by heat is effected at a temperature between about 350° F. and 475° F.

7. The method of producing an impregnated darkened wooden member as recited in claim 4, in which said wood is pine, and said darkening of the wood by heat is effected at a temperature between about 350° F. and 400° F.

8. The method of producing an impregnated darkened wooden member as recited in claim 4, in which said wood is fir, and said darkening of the wood by heat is effected at a temperature between about 375° F. and 425° F.

9. The method of producing an impregnated darkened wooden member as recited in claim 4, in which said wood is birch, and said darkening of the wood by heat is effected at a temperature between about 380° F. and 430° F.

10. The method of producing an impregnated darkened wooden member as recited in claim 4, in which said resin, after curing and after said darkening of the wood by heat, is transparent and thereby renders the grain of the darkened wood clearly visible through the resin.

11. The method of producing an impregnated darkened wooden member as recited in claim 4, in which said thermosetting resin is cured by heating to a temperature which is superatmospheric but is less than the temperature subsequently used for darkening the wood.

12. The method of producing an impregnated darkened wooden member as recited in claim 4, in which said impregnation of the wood with said resin is effected by immersing the wood in a body of uncured resin, and applying said superatmospheric pressure to said body of the resin to force it into the pores of the wood.

13. The method of producing an impregnated darkened wooden member as recited in claim 4, including the step of evacuating air and volatile constituents from the pores of the wood, prior to impregnation, by heating the wood and subjecting it to a vacuum, said impregnation of the wood with resin then being effected by immersing the wood in a body of uncured resin, and

14. The method of producing an impregnated darkened wooden member as recited in claim 4, including the step of evacuating air and volatile constituents from the pores of the wood, prior to impregnation, by heating the wood and subjecting it to a vacuum, said impregnation of the wood with resin then being effected by immersing the wood in a body of uncured resin, and

applying said superatmospheric pressure to said body of resin to force it into the pores of the wood.

References Cited in the file of this patent

UNITED STATES PATENTS

|           |          |                  |           |
|-----------|----------|------------------|-----------|
| 117,393   | Dunham   | July 25, 1871    | 1,723,384 |
| 921,000   | Roberts  | May 11, 1909     | 1,729,056 |
| 949,671   | Baekelan | Feb. 15, 1910    | 1,732,419 |
| 1,235,895 | Herbein  | Aug. 7, 1917     | 2,140,981 |
| 1,483,733 | Kozelek  | Feb. 12, 1924 10 | 2,398,649 |

|              |                |
|--------------|----------------|
| Snelling     | Aug. 6, 1929   |
| Texier       | Sept. 24, 1929 |
| Rice         | Oct. 22, 1929  |
| Booty et al. | Dec. 20, 1938  |
| Kvalnes      | Apr. 16, 1946  |
| Stover       | Nov. 18, 1947  |
| Bilhuber     | Nov. 14, 1950  |
| Austin       | Apr. 8, 1952   |
| Dannenberg   | Aug. 24, 1954  |
| McLaughlin   | Apr. 30, 1957  |